

## UNITED STATES PATENT OFFICE

EDWIN SUTERMEISTER AND JOSEPH A. WARREN, OF WESTBROOK, MAINE, ASSIGNEES  
TO S. D. WARREN COMPANY, OF BOSTON, MASSACHUSETTS, A CORPORATION OF  
MASSACHUSETTS

## PAPER MANUFACTURE

No Drawing.

Application filed April 7, 1928. Serial No. 268,367.

Our invention relates to the manufacture of sized and filled paper. We employ herein the words "sized" and "sizing" to define a treatment of paper in its manufacture which 5 renders an otherwise bibulous paper web relatively resistant to absorption of liquid, such as writing ink.

Furthermore our invention has for its object the employment as filling material for 10 sized paper the alkaline compounds of alkaline earth metals, of which calcium carbonate is an example; and which, if introduced into paper material in the beater with the usual rosin size, so acts as to defeat the ultimate object which is to produce an acceptable filled and sized paper. Heretofore it has been found impracticable to employ any of the said compounds as filler materials for 15 sized paper; our invention herein described 20 is characterized by the association with such material as calcium carbonate and the other ingredients of a batch of paper of a corrective or protective material which will enable the paper to be properly filled with the 25 minuted solid material and at the same time adequately and acceptably sized.

In the specification which follows, two examples of preparation and manipulation of 30 characteristic materials are given in detail.

Since precipitated calcium carbonate in 35 the form of waste lime mud is immediately available to many paper manufacturers that material is selected for the illustrations.

## EXAMPLE No. 1

35 *Preparation of sizing material and protective emulsion (parts and proportions by weight)*

Mix 1500 parts rosin with 225 parts sodium 40 carbonate in sufficient water to facilitate agitation and cook this with live steam until all of the carbon dioxide has been driven off. To this add 900 parts melted paraffin and, preferably, 100 parts sodium silicate, (the sodium 45 silicate is not indispensable but it has been found to assist in the production of emulsion). Stir the mixture thoroughly and then run it through a colloid mill, or otherwise treat it to produce thorough emulsion of the 50 paraffin.

*Preparation of lime mud (CaCO<sub>3</sub>)*

Take a wet lime mud containing 200 parts of CaCO<sub>3</sub> and about the same quantity of water and add to this as much of the above described emulsion as will contain 1½ parts paraffin and after mixing thoroughly add also 3.75 parts of alum in water solution. For 55 alum there may be substituted that quantity of aluminum hydrate as would be produced by converting the 3¾ parts of alum to hydrate. Grind this mixture for a time in a pebble mill, or otherwise agitate.

In the beater provide a batch containing 50 parts fibre (for instance half sulfite fibre and half soda fibre) with the usually proportionate quantity of water. To this add an ordinary rosin size emulsion in quantity to provide ¼ part rosin, then add ½ part alum. The foregoing materials having been thoroughly worked and mixed in the beater, add the lime mud preparation above described in such quantity as to supply 30 parts of CaCO<sub>3</sub>. This filler material as prepared should be 60 added in the wet state; if it has been allowed to dry the water-repellent characteristic of the CaCO<sub>3</sub> would render it extremely difficult to rewet and mix the material in the beater. When the above described filler material has been duly distributed and mixed 65 in the beater, add a solution containing 3 parts of alum as convenient before the batch of paper stuff is ready to be run out on the paper machine.

## EXAMPLE No. 2

70 *Preparation of rosin size and paraffin emulsion as prescribed for Example No. 1*

Start the beater batch as before with 50 parts of fibre and then put in a quantity of wet lime mud equivalent to 30 parts dry CaCO<sub>3</sub> and at the same time a sufficient quantity of the rosin size and paraffin emulsion to provide one part of paraffin. When these materials have been thoroughly mixed by the beater action, then add 6 parts alum, in solution, before the batch is run on the paper machine.

The paraffin emulsion in either of the illustrative examples above recited forms a pro- 75 80 85 90 95 100

tective barrier around or over the otherwise detrimental  $\text{CaCO}_3$  particles to such an extent that they do not react as they otherwise would to prevent the production of a properly 5 and truly sized paper. The quantitative proportions of materials hereinabove given are such as we know to be effective; these proportions can doubtless be varied and constituent quantities diminished in the interest of 10 economy without defeating the main object.

We claim:

1. Method of manufacturing filled and sized paper, characterized by the employment as a filler of an alkaline compound of an 15 alkaline earth metal in association with emulsified paraffin and rosin as a size.
2. Method of manufacturing filled and sized paper, characterized by the employment as a filler or calcium carbonate in association with emulsified paraffin and rosin as 20 a size.
3. Method of manufacturing filled and sized paper, characterized by the employment as a filler of an alkaline compound of an 25 alkaline earth metal associated with emulsified paraffin and rosin as a size, and the addition of alum as a final step in the beater.
4. Method of manufacturing filled and sized paper, characterized by employment 30 as a filler of calcium carbonate in association with emulsified paraffin and rosin as a size, and the addition of alum as a final step in the beater.
5. Sized paper containing as a filler an alkaline compound of an alkaline earth metal, 35 associated with paraffin and rosin as a size.
6. Sized paper containing as a filler calcium carbonate, associated with paraffin and rosin as a size.

40 Signed by us at Westbrook, Maine, this fifth day of April, 1928.

EDWIN SUTERMEISTER.  
JOSEPH A. WARREN.

45

50

55

60